

# UNITED STATES PATENT OFFICE.

ROBERT C. HARTONG, OF AKRON, OHIO, ASSIGNOR TO GOODYEAR TIRE & RUBBER COMPANY, OF AKRON, OHIO, A CORPORATION OF OHIO.

## PROCESS OF PRODUCING RUBBER COMPOSITIONS AND VULCANIZATION PRODUCT THEREFROM.

1,301,693.

Specification of Letters Patent. Patented Apr. 22, 1919.

No Drawing.

Application filed March 30, 1917. Serial No. 152,525.

To all whom it may concern:

Be it known that I, ROBERT C. HARTONG, a citizen of the United States, residing at Akron, in the county of Summit and State 5 of Ohio, have invented a new and useful Process of Producing Rubber Compositions and Vulcanization Product Therefrom, of which the following is a specification.

My invention relates to the art of producing rubber compositions and will be fully understood from the following specification. In the manufacture of rubber products a large variety of ingredients are employed and in every instance it is desirable to secure 15 a uniform and homogeneous mixture of these ingredients, both with one another and with the rubber, in order that the vulcanized product may be of highest quality. My invention is particularly concerned with a 20 method of procedure by which the ingredients of the composition may be incorporated into and disseminated through the rubber mix in the finest, practical state of subdivision and in such a manner as to secure true 25 homogeneity. This end I find to be best attained by the use of a liquid carrier for the ingredients.

It is a well understood fact that the action 30 of a solvent liquid upon a solid is to disintegrate that solid and break it up into excessively small particles, these particles when disseminated through the liquid being said to dissolve therein. For example it is believed that some substances of which the 35 soluble carbohydrate sugar may be taken as an illustration, disintegrate into their ultimate molecules in the presence of a sufficiently large volume of water, so that in a sugar solution the sugar exists in the most 40 extreme state of physical subdivision of which it is capable. Other substances, such as glue for instance, when dissolved in water do not appear to be subdivided to the same extent as the sugar particles mentioned, but 45 on the other hand they enter into some species of combination with the water by which they become enormously swollen or distended and if subjected to a grinding action in this distended condition may be more finely 50 divided than is possible in handling the dry product. In still other instances there may

be a disintegrating action by the solvent not approaching the disintegrating action effected in the case of the sugar solution but nevertheless very decided, unaccompanied 55 by any noticeable combination of the solid with the solvent. Illustrations of this species of action are found in colloidal solutions of metals such as gold and platinum in water and in such materials as arsenic 60 sulfid, clay, and the like. Finally the solvent may have comparatively little disintegrating power upon the solid but nevertheless still shows a distinct power of maintaining the solid in a fine state of subdivision 65 when this subdivision has been effected, or at least of enormously decreasing the rate of association of the particles of a finely divided substance. Thus for example when coarse materials of the nature of barytes are 70 suspended in water, each individual particle is retained in its separate state, agglomeration of the particles being prevented so long as the water is present in reasonable amounts.

It is therefore true that a carrier liquid 75 is in general useful to some extent, either in effecting disintegration of a solid substance or preventing or retarding the reassociation of disintegrated particles which have been reduced to a fine state of subdivision by any 80 means. From this standpoint alone therefore the use of a carrier liquid is advantageous in the mixing of rubber compositions. A further important advantage arises from the fact that the liquid carrying 85 the solid with it may be disseminated through the rubber with a relatively small amount of mechanical working, thereby avoiding the breaking down and loss of tensile strength of the rubber which results 90 from the excessive working sometimes necessarily resorted to in order to effect thorough dissemination of a solid constituent. The carrier liquid is also of particular advantage 95 in the case of solid ingredients which form true solutions such as the sugar solution mentioned, or which form colloidal solutions either as emulsion colloids or as suspension colloids and where relatively small percentages of the particular ingredients 100 are employed. By the increase in bulk or volume resulting from the action of the

carrier liquid the difficulty of effecting thorough dissemination of these relatively small percentages through the mass of the rubber mix is substantially lessened.

- 5 I have found that for the majority of materials employed for mixing with the rubber gum in the manufacture of rubber products, water forms the most desirable carrier liquid, both because of its cheapness  
 10 and because of the fact that it does not act upon the rubber in the mix. It must be understood, however, that other carrier liquids may be employed without departure from the basic principles of my invention.  
 15 After the mix has been satisfactorily made the water or other carrier liquid must be removed, it being well known that any large percentage of vaporizable matter such as water in the ordinary rubber mix is highly  
 20 disadvantageous in that vapors are evolved during vulcanization and the vulcanized product is thereby rendered porous. I find that the water may readily be removed, however, either by vacuum drying or by the use  
 25 of a current of air or other inert gas, the expense of the treatment being far outweighed by the advantages resulting from the use of the carrier liquid in mixing the composition.  
 30 As specific examples of the uses to which my invention may be put the following may be enumerated.

#### *Alumina.*

- 35 It is difficult to secure satisfactory results with alumina as a composition ingredient by the ordinary methods employed for disseminating it through the mass. If, however, the alumina be suspended in water in the form  
 40 of hydrate of alumina ( $Al(OH)_3$ ), this hydrate is more or less colloidal in character and in consequence is in a much finer state of subdivision than the oxid itself may be reduced to. By incorporating such a water  
 45 suspension of aluminum hydroxid in a rubber mix I secure a perfectly homogeneous mass, and the water having been removed previous to vulcanization, as by vacuum drying, the vulcanized product evidences in all  
 50 of its physical properties the more perfect nature of the mixing process.

#### *Colloidal metals.*

- What has been said of alumina is also  
 55 quite true of certain metals, such as iron and lead. These metals, when reduced to a very fine powder by grinding, do not become composition ingredients which have any great commercial value. If, however, these metals  
 60 are obtained in colloidal form and are added to the rubber in the form of a thick paste, using water or a dilute colloidal solution of glue or gelatin as the liquid medium; the moisture subsequently removed by drying  
 65 before the other ingredients are added; a

very decided improvement will be obtained in the quality of the finished product.

#### *Barytes.*

It has long been known that barytes prepared by grinding the mineral as found in nature is inferior to barytes precipitated from an aqueous solution, in the manufacture of rubber products, this inferiority being due to the imperfect subdivision of the material effected by dry grinding. The advantages gained by the initial precipitation are to a large extent lost, however, by the subsequent drying of the precipitate, the fine particles agglomerating or reassociating to a considerable extent so that while they remain finer than the dry-ground product they are nevertheless relatively coarse as compared with the suspended precipitate. In accordance with my invention I may avoid the reassociation of the finely divided suspended precipitate by incorporating the original suspension directly in the rubber mix. By the use of the precipitate as prepared in a dilute solution, the fineness of the precipitate being to a considerable extent a function of the dilution, even better results may be secured. A further improvement may be effected by adopting measures to prevent the coalescence of the precipitate within the solution or suspension. This effect may be obtained by causing the precipitation to take place in the presence of glue, gelatin or similar emulsion colloids. The action of such colloids appears to be similar to that of an emulsifying agent, the nascent particles of the precipitate being instantly coated with the glue or the like, which coating serves to prevent coalescence.

#### *Glue.*

105 The alumina and barytes previously mentioned may be called irreversible colloids in that the particles should be retained in the solution in which they are produced until the completion of the mixing process in order to prevent their coalescence into larger masses which could not again be reduced to the form of a suspension colloid or suspensoid without considerable manipulation. On the other hand materials such as animal glue may be called reversible colloids, in that after having been reduced to the solid form they may be again converted into emulsions by the simple addition of water.

110 Commercial glue reduced to the finest state of subdivision possible by dry grinding is unsatisfactory as a constituent of the rubber composition in that it is practically impossible to secure a mixture so homogeneous that small particles of the glue will not remain visible upon examination under the microscope. If, however, this glue be treated with water so that it becomes swollen and forms a gel, perfect mixing may be 115 120 125 130

effected by the ordinary methods and examination of the final product either before or after vulcanization fails to show any lack of homogeneity. Furthermore it is possible by 5 this method of producing the mixture to secure a final vulcanized product exhibiting physical properties unobtainable by the known methods.

My invention is particularly valuable in 10 the employment of gel-forming emulsoids such as glue as compounding ingredients in that the particles which are once separated from one another in mixing have no tendency to again coalesce should they adventitiously come into contact at some later stage of the mixing.

*Zinc oxid and other insoluble, non-colloidal, unemulsifiable compounding ingredients.*

20 The use of a carrier liquid with such ingredients as zinc oxid would appear to involve no action other than the purely physical one of facilitating the dispersion of the solid through the mixture. The technical 25 results and advantages which follow from this purely physical action are however of considerable importance and warrant the use of my invention for mixing ingredients such as those named upon which the carrier liquid 30 exerts little or no dissociating action. If such materials be incorporated into the rubber mix by the known methods the most thorough mechanical manipulation or kneading of the mix must be resorted to to 35 effect any satisfactory dissemination, the material tending to associate itself into lumps which must be most carefully broken up if a high grade product is to be obtained. On the other hand long continued mixing 40 or kneading operations tend to affect the properties of the rubber gum itself in an injurious manner and a nice balance must therefore be maintained between unsatisfactory mixing and overworking.

45 By the use of a carrier liquid serving as a dispersing medium for these ingredients entirely satisfactory results can be secured and all danger of overworking the rubber is obviated. It is not necessary in the use of 50 zinc oxid or the like to employ large quantities of the carrier liquid, an amount of liquid sufficient to form a semi-fluid paste being quite sufficient for practical purposes.

While I have described in considerable detail 55 the theories which I believe to underlie my invention, and have set forth the specific manner of operation and some of the results which can be obtained in the use of specific constituents according to the invention, it 60 will be understood that my invention is not dependent upon the soundness of the theories which I have advanced nor limited to the specific materials or methods of manipulation named, except in so far as such limitations are included within the terms of the

accompanying claims in which it is my intention to claim all novelty inherent in my invention as broadly as is permissible in view of the prior art.

What I claim as new and desire to secure 70 by Letters Patent is:—

1. The process of forming a rubber composition which consists in adding to rubber a volatilizable carrier liquid holding a composition ingredient in a fine state of subdivision, mixing the carrier liquid and the ingredient held thereby with the rubber, volatilizing the carrier liquid, whereby the ingredient is left disseminated throughout the mix, and heating the mix with a vulcanizing agent to effect vulcanization. 75

2. The process of forming a rubber composition which consists in adding to rubber, water holding a composition ingredient in a fine state of subdivision, mixing the water 85 and the ingredient held thereby with the rubber, volatilizing the water, whereby the ingredient is left disseminated through the mix and heating the mix with a vulcanizing agent to effect vulcanization. 90

3. The process of forming a rubber composition which consists in adding to rubber a colloidal solution of a composition ingredient, mixing the solution with the rubber, volatilizing the solvent, whereby the ingredient is left disseminated through the mix, 95 and heating the mix with a vulcanizing agent to effect vulcanization.

4. The process of forming a rubber composition which consists in adding to rubber 100 a composition ingredient in the condition of a gel, mixing the gel with the rubber, volatilizing the solvent from the gel whereby the ingredient is left disseminated through the mix, and heating the mix with a vulcanizing agent to effect vulcanization. 105

5. The process of forming a rubber composition which consists in adding to rubber a proteid in solution, mixing the solution with the rubber, volatilizing the solvent 110 whereby the proteid is left disseminated through the mix, and heating the mix with a vulcanizing agent to effect vulcanization.

6. The process of forming a rubber composition which consists in adding to rubber 115 a solution of animal glue, mixing the solution with the rubber, volatilizing the solvent whereby the glue is left disseminated through the mix, and heating the mix with a vulcanizing agent to effect vulcanization. 120

7. The process of forming a rubber composition which consists in adding to rubber a wet precipitate of a composition ingredient, which precipitate has been formed in the presence of a protective colloid, mixing 125 the resultant precipitate with the rubber, drying the mix, and heating the mix with a vulcanizing agent to effect vulcanization.

8. The process of forming a rubber composition which consists in adding to rubber 130

a wet precipitate of barium sulfate, which precipitate has been formed in the presence of a colloidal gel, mixing the resultant precipitate with the rubber, drying the mix, 5 and heating the mix with a vulcanizing agent to effect vulcanization.

9. The process of preparing a composition ingredient for rubber products, which consists in precipitating such ingredient 10 from a solution containing a gel-forming colloid, whereby the nascent precipitate is coated with gel.

10. The method of preparing barium-sulfate for use as a composition ingredient 15 in rubber products which consists in precipitating the barium-sulfate in a solution containing animal glue, whereby the nascent precipitate is coated with glue.

11. The process of forming a rubber composition which consists in adding to rubber a composition ingredient in the form of a precipitate carried by the liquid in which it was precipitated, mixing the carrier liquid 20 and the precipitate with the rubber, vola-

tilizing the liquid, and heating the mix with 25 a vulcanizing agent to effect vulcanization.

12. The homogeneous vulcanized product formed by adding to rubber a composition ingredient in a fine state of subdivision and held by a carrier liquid, mixing the liquid 30 and ingredient held thereby with the rubber, driving off the liquid and heating the resultant dry mix with a vulcanizing agent to effect vulcanization.

13. The homogeneous vulcanized product 35 formed by adding to rubber a proteid held by a carrier liquid, mixing the proteid and carrier liquid with the rubber, driving off the carrier liquid, and heating the resultant dry mix with a vulcanizing agent to effect 40 vulcanization,

14. The homogeneous vulcanized product formed by adding to rubber animal glue 45 formed into a gel by water, mixing the gel with the rubber, driving off the water, and heating the resultant dry mix with a vulcanizing agent to effect vulcanization.

ROBERT C. HARTONG.